

May 8, 1928.

1,668,734

E. E. SCHUMACHER

ELECTRON EMITTING CATHODE AND METHOD OF MAKING IT

Filed July 12, 1923



Inventor:  
Earle E. Schumacher,  
by J. C. Palmer Atty

Patented May 8, 1928.

1,668,734

# UNITED STATES PATENT OFFICE.

EARLE E. SCHUMACHER, OF EAST ORANGE, NEW JERSEY, ASSIGNOR TO WESTERN ELECTRIC COMPANY, INCORPORATED, OF NEW YORK, N. Y., A CORPORATION OF NEW YORK.

## ELECTRON-EMITTING CATHODE AND METHOD OF MAKING IT.

Application filed July 12, 1923. Serial No. 650,985.

This invention relates to electron emitting cathodes and has for its object a filament of high thermionic activity.

This object is attained by combining a thermionically active material with a metallic filament. To do this, the filament is heated to at least a red heat, preferably in vacuum, and finely powdered thermionically active material is brought into contact with the surface of the filament. The powder adheres to the filament and is incorporated therewith to form a highly active and stable cathode. A filament of tungsten, molybdenum or the like may have alloyed, by this method, a thermionically active metal, such as uranium or the metals of the cerium group. Cathodes having these constituents possess a thermionic activity comparable to that of a platinum nickel filament coated with alkaline earth oxides.

Referring now to the drawing, the single figure thereof discloses an apparatus for treating filaments.

Within an evacuated vessel 10 is supported, by means of leading-in wires 11 and 12 sealed in the vessel, a metallic filament 13, which is to be treated. Also contained within the vessel 10 is a supply 14 of a thermionically active material to be combined with the filament 13, the material being in finely powdered condition. A battery 15 is connected to the leading-in wires 11 and 12 to provide heating current for the filament.

After the filament has been mounted without in the vessel and the powdered thermionically active material introduced, the vessel is evacuated. The filament 13 is then heated to a red heat, or hotter if necessary, and the vessel 10 shaken to bring the particles of the thermionically active material into contact with the surface of the filament. The particles contacting with the filament adhere thereto and combine therewith to form a composite filament. After sufficient of the powdered material has been combined with the filament, the current is cut off, the vessel opened and the filament removed therefrom. The filament is then combined with the other elements of an electron discharge device and sealed within an evacuated vessel in the usual manner.

This method of producing thermionic cathodes is particularly adapted for use in forming an alloy filament of tungsten,

molybdenum or other metals capable of being formed into a filamentary conductor and thermionically highly active metals, such as cerium, lanthanum, praseodymium, neodymium, samarium or uranium. The latter metals may be introduced into the vessel 10 in the form of filings. The metallic filament is heated to a sufficiently high temperature so that when the filings come in contact therewith, they combine therewith to form an alloy. The temperature of the filament may range from a dull red heat up to white hot, depending upon the particular filament used and the extent of oxidation of the metal filings. If the filings are considerably oxidized, the filament has to be more highly heated than otherwise. An alloy filament formed of tungsten or molybdenum, and any one of the afore-mentioned thermionically active metals, possess a thermionic activity comparable to that of a platinum nickel filament coated with alkaline earth oxides.

Although this invention has been disclosed as particularly adapted for forming metallic filaments, the method employed is adapted for use wherever it is desired to combine any thermionically active material with a conductive core. For example, this method is also capable of use in the production of metallic filaments coated with alkaline earth oxides. A filament of tungsten, tantalum, molybdenum, or the like, may have applied thereto a coating of barium and strontium oxides or other similar alkaline earth oxides by providing a supply of the coating material within the vessel 10 and shaking the latter to bring the powdered material into contact with the heated filament. The particles will adhere to the filament and form therefor a thermionically highly active coating.

The selection of materials to be combined, according to this method, is therefore not limited to the particular materials above enumerated and various materials may be utilized without departing in any way from the spirit of the invention, as set forth in the appended claims.

What is claimed is:

1. The method of producing a thermionic cathode which comprises supporting a metallic filament in an evacuated vessel containing powdered thermionically active material, passing heating current through said

filament, and agitating said vessel to bring said thermionically active material into contact with said heated filament.

2. The method of producing a thermionic cathode which comprises heating a metallic filament and bringing powdered thermionically active material into contact therewith under the influence of gravity only.

3. A method of producing a thermionic

cathode which comprises supporting a filament in a vessel containing thermionically active material, heating said filament and bringing said thermionically active material into contact with said filament under the influence of gravity only. 10

In witness whereof, I hereunto subscribe my name this 3rd day of July, A. D. 1923.

EARLE E. SCHUMACHER. 15